

## UNITED STATES PATENT OFFICE

2,253,655

## COATED OR IMPREGNATED PAPER PRODUCT AND METHOD OF MAKING SAME

Frederick Shurley, Salt Lake City, Utah, assignor  
to Crown Cork & Seal Company, Inc., Baltimore, Md., a corporation of New York

No Drawing. Application April 1, 1936,  
Serial No. 72,207

6 Claims. (Cl. 91—68)

This invention relates to a composition of matter which may be applied to paper or paper-like materials and has particular application as a coating for, or ingredient of, paper employed in making receptacles adapted to contain milk, and closures therefor. The invention also relates to the method of preparing and applying this composition and the resulting material.

It has been found that, when paper or like material is subjected to the action of milk, the casein in the latter will react with the paper resulting in the formation of a gummy, adhesive-like substance. This is always objectionable and particularly so since it causes paper milk bottle caps to stick tightly to the tops of the bottles, or other containers. The sticking or gumming of the inner surface of the caps results in tearing of the paper when the cap is removed and prevents reuse of the caps to again cover the product in the container.

Various coatings, as for example, paraffin and other waxes, have been heretofore used in an attempt to overcome this condition, but have not met with success, owing to an objectionable reaction between the casein of the milk and the wax.

It has been found that by the use of the composition herein described, either as an ingredient of the paper or as a coating for the paper, the above mentioned difficulties may be overcome.

Other advantages of this composition over waxes and similar coatings reside in its enhanced lubricating power which prevents the paper from breaking as frequently occurs in the dry die forming out of tops and bottoms of cylindrical containers, drinking cups, cardboard pie plates, and similar articles from the blank material. In addition, the composition bodies and revitalizes the paper, so that its shape is permanently retained. A particular advantage of the composition is that it does not stain paper and may be successfully used on substantially any type of paper.

The composition reduces the surface tension of all water soluble materials, and because of its penetration into the fibre, it makes the paper more flexible. It also aids the dispersion of pigments, dyestuffs and coloring matter, causing them to spread more evenly and uniformly, and insuring a proper penetration. Furthermore, the composition is not toxic or in any way injurious to food products and has no disagreeable odor.

It will be understood that the invention is not confined to the treatment of materials which are to be used for containers or closures, but as an

illustrative embodiment of the invention the production of such articles will be described.

In the manufacture of paper milk bottle caps, cap linings, or paper containers, the paper may be first coated with a composition having the following formula:

|                        |         |   |
|------------------------|---------|---|
| Water                  | gallons | 1 |
| Glyceryl mono-stearate | ounces  | 4 |
| Glycerol               | do      | 2 |

The water acts as the carrier or base for the other ingredients. The glyceryl mono-stearate contributes the lubricating, plasticizing, bonding, and casein resisting properties of the product, and the glycerol acts as an emulsifier and makes possible the production of a colorless, spreadable, penetrating, and non-staining product.

Although not essential, it may be desirable to add to the above composition about 10 grams of "Lohrinol," (the trade name of a product consisting of sodium lauryl sulphonate sold by Glyco Products Co., Inc.) which will tend to increase the penetrating and spreading qualities of the composition and about 5 grams of benzoate of soda which will act as a preservative.

The above composition is prepared by heating the water to approximately 55° C., adding the Lohrinol, (if used) and stirring until solution is effected. The glycerol is then added, and following the addition of the glycerol, the glyceryl mono-stearate is added. The preservative (if used), may be added before or with the addition of the glyceryl mono-stearate. The mixture is stirred during the addition of these ingredients, and stirring is continued until the ingredients have emulsified. The temperature is maintained at approximately 55° C., until the emulsification has been completed, after which the heat is removed. During the subsequent cooling, the stirring is continued to prevent separation, and a white product of butter-like consistency will result.

In preparing the composition, I sometimes find it desirable to add about 2 grams of vanillin or other flavoring material to give the otherwise odorless product a pleasant aroma.

I have referred above to the preferred quantities of ingredients used in preparing this composition, but I find that from 3 to 8 ounces of the glyceryl monostearate and from 2 to 4 ounces of the glycerol, when added to 1 gallon of water, will give satisfactory results. Obviously, the quantities of the non-essential ingredients, such as "Lohrinol" and the preservative, may be varied within wide limits.

It will be understood that equivalents may be substituted for the above mentioned ingredients. For example, in place of glyceryl mono-stearate, I may use an equal amount of glycol stearate and in place of glycerol, I may use an equal amount of liquid petrolatum, triethanolamine, or "Glycopon," (the trade name of a product consisting of a mixture of polyhydric alcohols sold by Glyco Products Co., Inc.).

The composition may be applied by coating the paper or paper-like material as by means of rollers, or by brushing, or spraying.

In some cases, it is preferable to incorporate the composition in the paper during the manufacture of the latter by mixing it in suitable proportions with the paper pulp prior to the drawing or screening of the paper. It has been found that the composition when so used bonds very effectively in the paper.

Where the product is used in connection with containers for food it is usually essential that it be odorless or that such odor as may be present be a pleasant one and the above described composition meets this requirement. However, when the presence or absence of an odor is immaterial it is possible and may be desirable to use, in place of the glyceryl mono-stearate, equal quantities of glyceryl di-stearate, glyceryl tri-stearate, triethanolamine stearate or trihydroxyethylamine stearate (sold by Glyco Products Co., Inc.).

The above described composition may be used in the preparation of ceramic products as a temporary binder for molded clay articles such as firebricks, prior to fusing, firing or baking, enabling the clays to be molded without crumbling. The advantages of the use of this composition for such a purpose are due to its water dispersability, and the fact that it, being completely organic, leaves no residue on firing. The quantity which is added is not critical, but is generally determined merely by adding the composition to the clay with mixing until the desired plastic consistency is obtained.

The composition also serves as an excellent binder for abrasive materials in the manufacture of solid articles, such as abrasive wheels, due to its water dispersability and its completely organic nature. It may be compounded with abrasive material in any convenient proportions to form a plastic moldable article and upon heating, firing or fusing the article, the binder volatilizes and completely disappears.

I claim:

1. Paper treated with a composition comprising glycerol and a substance selected from the group consisting of the glyceryl stearates, glycol stearates, triethanolamine stearate and trihydroxyethylamine stearate.
2. Paper treated with a composition comprising glycerol and glyceryl mono-stearates.
3. A method of treating paper which comprises applying thereto a composition comprising glycerol, a substance selected from the group consisting of the glyceryl stearates, glycol stearates, triethanolamine stearate and trihydroxyethylamine stearate, and water and thereafter drying.
4. Paper treated with a composition comprising glycerol, sodium lauryl sulphonate and a substance selected from the group consisting of the glyceryl stearates, glycol stearates, triethanolamine stearate and trihydroxyethylamine stearate.
5. Paper treated with a composition comprising glycerol, sodium lauryl sulphonate and glyceryl mono-stearates.
6. A method of treating paper which comprises applying thereto a composition consisting of glycerol, sodium lauryl sulphonate, and a substance selected from the group consisting of the glyceryl stearates, glycol stearates, triethanolamine stearate and trihydroxyethylamine stearate, and water and thereafter drying.

FREDERICK SHURLEY.